

Jan 6, 1931.

J. A. KENNEDY

1,787,629

NONSTICKY WATER AND FLAME RESISTANT INSULATED CONDUCTOR,  
CONDUIT, ETC., AND METHOD OF MAKING

Filed Oct. 2, 1928



Fig. 1.



Fig. 2.



Fig. 3.



Fig. 4.

Fig. 5.

Inventor  
Joseph A. Kennedy  
by Wright, Brown, Dunphy, Tracy  
Attn:

## UNITED STATES PATENT OFFICE

JOSEPH A. KENNEDY, OF PAWTUCKET, RHODE ISLAND, ASSIGNOR, BY MESNE ASSIGNMENTS, TO ANACONDA WIRE AND CABLE COMPANY, A CORPORATION OF DELAWARE

NONSTICKY WATER AND FLAME RESISTANT INSULATED CONDUCTOR, CONDUIT, ETC., AND METHOD OF MAKING

Application filed October 2, 1928. Serial No. 309,802.

This invention relates to the art of water-resistant and flame-proofed insulated electrical cable and other conductors, non-metallic flexible conduit for receiving and protecting electrical conductors, and other manufactures of similar character. It is concerned with methods of treating such manufactures to make them not only water-proof and flame-proof within the limits of established practice, but also non-sticky on the surface.

Such goods are treated with compounds to render them water-proof and flame-proof, conforming to the standards established by the National Board of Fire Underwriters.

Heretofore asphaltum has been commonly used as the water-proofing compound, and stearin pitch as the flame-proofing compound, the asphalt being first applied and caused to penetrate and impregnate to a greater or less extent the sheathing of the conductor cable or the structure of the conduit, and the stearin pitch being subsequently applied as an outer coating. While these substances are satisfactory from the point of view of the underwriters' requirements and cost considerations, the stearin pitch coating has the objectionable quality of being sticky. It is a semi-solid amorphous substance when cold, and is liquefiable by heat. It is applied to the goods by passing the latter through a body of the stearin pitch contained in liquid condition in a heated tank. After heating and application in this manner, its sticky condition persists even after cooling, so that when the coated goods have been rolled into a coil for storage and shipment, the turns of the coil adhere together and the coating is liable to be more or less stripped off when uncoiled; and also the sticky material soils

the hands of users and anything else with which it may come in contact. In the effort to overcome this sticky quality, the practice has been commonly followed of passing the coated goods, after leaving the tank of melted stearin pitch, through a loose mass of mica flakes or powdered talc, some of which will adhere more or less firmly to the sticky coating. But the protection given by this means is not complete and satisfactory. Another effort in the same direction, which consists

in applying an additional coat of paraffin or other waxy substance over the stearin pitch has met with greater success. Both of these treatments, however, involve material, and a step in the process, additional to the commonly used asphaltum and stearin pitch, and to the processes followed in applying these substances.

According to the present invention, I obtain the desired effect of water-proofing and flame-proofing the goods, and overcoming the stickiness of the flame-proofing coat, by successive treatments with wax and stearin pitch, eliminating the use of asphaltum altogether and the step of applying powdered mineral or melted wax on the surface of the flame-proofing compound. In this new treatment the wax impregnation takes the place of asphalt impregnation and obtains an equally successful water-proofing effect. It likewise neutralizes or overcomes the surface stickiness of the stearin pitch coat. The last named effect is due to the fact, which I have discovered and utilized industrially for the first time, I believe, that when wax of lower melting point than stearin pitch is applied as an impregnating agent and afterwards the impregnated article is covered with hot stearin pitch, a small proportion of the wax will penetrate the stearin pitch coating to the outer surface. The amount of wax which thus penetrates is sufficient to neutralize the adhesive quality of the external surface of the stearin pitch coating and produce a waxy feeling to the touch, but is insufficient to increase the inflammability of the stearin pitch coat appreciably. It does not exist on the surface of the pitch coating as a distinct film of wax.

The steps of the process and characteristics of the product in which this invention resides are more fully described in the following specification, in connection with the drawings. In the latter,

Figs. 1, 2 and 3 are diagrammatic views illustrating the nature of the steps performed in impregnating a cable or electrical conductors according to this invention but without attempting to show the details of the commercial apparatus employed;

Fig. 4 is a fragmentary elevation of a partially dismembered cable embodying this invention;

Fig. 5 is a fragmentary partial elevation and 5 partial section of a conduit for electrical purposes embodying the same invention.

The invention may be applied to the treatment of all types of flexible insulated electrical conductors or cables, and flexible non-metallic conduit designed to receive electrical conductors and for like uses. In Fig. 4 I have shown illustratively a cable consisting of two insulated wires *a* and *b* which are wrapped about with strands of twisted paper or 10 other equivalent cords in order to preserve and maintain a prescribed distance between the metallic cores of the individual conductors, and are laid side by side, in conjunction with thick filler cords *d*, *d*, into a cable which 15 is covered by a sheath *e* constructed of interwoven or braided strands. In Fig. 5 I have shown a flexible non-metallic conduit of the type shown in the Smith Patent No. 1,016,527, February 6, 1912, as illustrative of another 20 class of goods in which the invention may be embodied, such conduit being constructed of longitudinal warp strands and helical weft or filling strands.

In applying the treatment of this invention 25 to a cable, the separate wires, with their surrounding strands *c*, are passed through a tank *h* containing a body of melted wax and heated by gas flames *i* or otherwise to a temperature high enough to keep the wax in melted condition. After the wax thus applied has 30 become solid, the wires are combined in a cable and covered with the woven or braided sheath *e*. The entire cable is then passed through a similar heated tank *j* containing 35 wax in melted condition. The wax is sufficiently fluid and the cable is passed through the tank slowly enough to permit a substantially 40 complete impregnation of the sheath and the component strands thereof by the wax. As 45 the cable emerges from the tank the surplus wax adhering to its surface is wiped off by means well understood in the art.

In these treatments I may use any wax 50 which has a melting point lower than that of stearin pitch and is sufficiently thin when melted to penetrate into and between the strands of the sheath, as above set forth. Paraffin wax is suitable for this purpose and 55 may serve as an illustration of a large class of equivalent waxes having the desired properties.

The procedure above described, so far as 60 concerns the preliminary treatment of the wires before being covered with the sheath *e*, may be modified or omitted without departure from the invention. Thus, in the case of 65 cables containing two or more wires differently colored to designate different polarity, the light colored wire or wires may be treated with a clear wax, and black or other dark

colored wires treated with a different suitable compound, if desired, to reduce expense or for other reasons. Or indeed the preliminary wax treating may be omitted altogether and the treatment after application of the sheath relied on to permeate the covering strands *c*, and even the braided jackets of the individual wires. 70

Finally the wax impregnated cable, after cooling, is passed through a tank *k* containing 75 a body of melted stearin pitch maintained in a sufficiently fluid condition, by the heat of gas flames under the tank or other suitable means, to permit immersion and passage of the cable through it. In leaving the tank 80 the cable passes through a die or wiper which removes the excess of stearin pitch. A second coat of stearin pitch may be applied if desired by a repetition of the step last described.

The heat of the stearin pitch bath melts the 85 previously applied wax; and the free melted wax, that is, so much of it as is not retained in the sheath by capillarity, percolates 90 through the enveloping coat or coats of stearin pitch and appears on the surface of the outer coat in sufficient quantity to give it a slightly waxy feeling to the touch and make it completely non-adhesive either to adjacent 95 bodies of the same material, to the hands of the user, or to other objects with which it may 100 come in contact. But the wax does not make a perceptible film on the surface, neither is it present in sufficient quantity to burn when subjected to the flame test, or to impair the 105 ability of the stearin pitch coating to conform to the established flame-proofing standards. It leaves the sheath highly flexible and avoids deposit of a black sticky compound on the inside of the sheath and on the individual wires. As the result of using wax in this 110 connection the stearin pitch coating does not penetrate through the meshes of the sheath and does not form a sticky layer on the inside 115 of the sheath, nor does it penetrate to the wires and discolor their surfaces. When such goods are treated by impregnation first in melted asphaltum and then in melted stearin pitch, the black compounds usually penetrate 120 the sheath more or less, leaving a sticky deposit on the inside of the sheath which soils the hands of the workman when removing the sheath preparatory to connecting up the wires, and also discoloring those wires which are given a light color for polarity distinction.

Conduits are treated according to this invention in the same way as above described with respect to cable. Indeed an open conduit of woven construction is essentially the same as the outer sheath of a cable or other insulated conductor, so far as the invention 125 is concerned. It differs in having an open interior instead of being filled with wires, etc., but it is so passed through the baths of wax and stearin pitch that these materials are applied to it on the outside only and pen- 130

etrate only to the extent that they can soak into the interstices during the time that a given point in the length of the conduit remains in the bath. The same qualities are given to the conduit by this treatment as are given to the cable. For the purpose of generic definition I have adopted the term "covering for electrical conductors" to designate both the conduit as a separate article of manufacture, and the outer sheath which receives the impregnating and coating treatment as a component of an electrical cable or single insulated conductor which may be treated by this method.

It will be noted that in the treatment of both described embodiments of such coverings, according to this invention, the usual coating or impregnation by asphaltum is omitted, and the water-proofing effect is fully and adequately obtained by the substituted wax treatment. Thus the wax performs the double function of water-proofing the article and mitigating the stickiness of the flame-proofing compound. And, in application according to my discovery and invention, it performs these functions without creating a fire hazard.

What I claim and desire to secure by Letters Patent is:

1. The method of water-proofing and flame-proofing coverings for electrical conductors which consists in first impregnating such covering with wax of a lower melting point than the after-mentioned flame-proofing compound, and then enveloping said covering with a coat of flame-proofing compound which is liquefiable by heat and is applied at a temperature higher than the melting point of the wax.

2. The method of water-proofing and flame-proofing coverings for electrical conductors, and mitigating the stickiness of the flame-proofing substance, which consists in first applying to the covering a waxy substance which is liquefiable at a temperature lower than that to which the flame-proofing substance is brought when applied to the covering, and also has the property of penetrating the flame-proofing substance when both are in the liquid condition; and then applying to the article thus treated a coating of flame-proofing composition at a temperature high enough to melt the waxy substance.

3. The method of water-proofing and flame-proofing coverings for electrical conductors, which consists in applying wax to such coverings, and then applying a coating of melted stearin pitch over the surface of the wax treated article, in fluid condition and at a temperature above the melting point of the wax, whereby the wax is caused to penetrate through such stearin pitch coating in sufficient quantity to mitigate the surface stickiness of the latter, when cooled to

the atmospheric temperatures, but insufficient to create a fire hazard.

4. A covering for electrical conductors having a water-proofing content of wax on and adjacent to its outer surface, and an enveloping coating of flame-proofing material interpenetrated to a certain extent by such wax.

5. A covering for electrical conductors constructed of interconnected fibrous strands having an outer coating of flame-proofing material which in itself is more or less sticky at ordinary temperatures, and having a content of wax within its structure inside of said coating and penetrating the latter to the outer surface in sufficient measure to render such surface substantially non-sticky.

6. A covering for electrical conductors of textile construction, combined with a wax impregnation and a flame-proofing coating of stearin pitch, a portion of the wax being interspersed through said coating to the outer surface thereof in sufficient measure to render such surface substantially non-sticky, but insufficient to create a fire hazard.

In testimony whereof I have affixed my signature.

JOSEPH A. KENNEDY.

70

75

80

85

90

95

100

105

110

115

120

125